

Oct. 11, 1938.

H. MATTHIES

2,132,858

**H. MATTHIES**  
**PROCESS OF CONTINUOUSLY PRODUCING ZINC IN VERTICAL  
REDUCING CHAMBERS AND APPARATUS THEREFOR**  
Filed June 9, 1937

Filed June 9, 1937

Fig. 1



Fig. 2  
(A-A)



*Inventor:*

HERMANN MATTHIES  
BY

BY  
A. PR. HELLER

ATTORNEY

## UNITED STATES PATENT OFFICE

2,132,858

PROCESS OF CONTINUOUSLY PRODUCING  
ZINC IN VERTICAL REDUCING CHAMBERS  
AND APPARATUS THEREFOR

Hermann Matthies, Duisburg-Wanheim, Germany, assignor to American Lurgi Corporation, New York, N. Y., a corporation of New York

Application June 9, 1937, Serial No. 147,174  
In Germany June 10, 1936

11 Claims.

(Cl. 75—86)

The present invention relates to a zinc reducing process, and, more particularly, to a process for the continuous production of zinc in vertical reduction chambers.

Heretofore, numerous attempts have been made to smelt raw materials containing zinc in vertical muffles in a continuous operation. Most of these prior attempts have completely failed due to various serious practical difficulties. Even the few methods which have attained some practical importance in comparison with the conventional smelting processes in the horizontal muffle, had very serious defects which rendered the production process difficult and expensive in practical operation.

In view of the good results obtained with silicon carbide as a highly refractory structural material of good heat conductivity, the important problem of providing a suitable structural material for muffles has been satisfactorily solved. However, another equally important problem still remained in the construction of vertical muffles, to wit: the satisfactory removal of the reduction gases from the heated muffle chamber into the condensing plant. Prior attempts of solving this problem involved internal, stationary, hollow or loosely filled structures in the muffle or briquetting and coking of the ore-coal mixture. None of these prior attempts was completely satisfactory or successful, or free from drawbacks and difficulties. The stationary internal structures became obstructed and were difficultly accessible for the purposes of inspection and cleaning. Briquetting and coking, on the other hand, were expensive and had to be determined by experiment for each kind of ore. Only suitably shaped solid ore-coal briquettes provided a sufficiently loose stratification in the vertical muffle for the removal of the gaseous products of reduction to the condensing plant. They also presented great resistance to the conduction of heat in consequence of the desired small number of contact points of small surface and thus greatly increased the cost of heating.

It has been found that the above problem may be solved in a simple and efficient manner.

It is an object of the present invention to provide an improved process for the production of zinc in vertical muffles which is free from the disadvantages of conventional processes.

It is another object of the present invention to provide a novel and improved process for the continuous production of zinc in vertical reduction chambers.

It is a further object of the present invention

to provide a vertical muffle of novel and improved character which is capable of continuously producing zinc from zinciferous material on a practical and industrial scale.

Other and further objects and advantages of the present invention will become apparent from the following description taken in conjunction with the accompanying drawing, in which:

Fig. 1 illustrates a vertical and longitudinal sectional view of a vertical reduction chamber embodying the principles of the present invention; and

Fig. 2 depicts a section taken on line A—A of Fig. 1.

Broadly stated, according to the principles of the present invention a vertical muffle is provided for the continuous production of zinc, said muffle having its upper portion divided in three chambers down to about the heating chamber by means of two vertical partition walls. Of these three chambers the middle one is charged with coarse granular pieces of a heat-resisting material forming no slag and which is not attacked by zinc vapors, the two chambers at each side of the center chamber are filled with a mixture of zinciferous materials and of a reducing agent. The zinc vapors produced in the heated portion of the muffle are removed into a condenser through the center column constituted of coarse pieces of an inert material extending downwards which due to its structure is readily permeable to gases, whereas the residues of the zinciferous charge and of the granular material containing no zinc may be withdrawn continuously or intermittently at the bottom of the reducing shaft.

It is generally preferred to provide a muffle shaft of quadrangular cross section and to divide the upper part thereof, for example the section located above the heating zone or a portion thereof, into three vertical chambers. In this manner one charging column lies against each of the two longitudinal walls of the shaft and a third column extending along the full height of the shaft in the core of the muffle is enclosed by these two lateral columns. These three charging columns are formed by the division of a section of the upper part of the muffle by means of two longitudinal walls carried by supporting arches provided within the muffle. The supporting arches, in this type of structure, are advantageously located directly above the heated muffle shaft so that the anchoring of the arches presents no difficulties. Preferably, at the same point, to wit: above the heated shaft

- chamber, an opening is provided in one muffle wall of the center shaft, which communicates with the condenser. However, this opening may be situated at a higher or lower level. The height of the part of the charging shaft which is divided into three chambers and is located above the heating chamber of the furnace, is preferably made so great that the preliminary drying of the charge and adequate heating are ensured.
- 10 The whole muffle shaft is preferably constructed of structural materials having good heat conductivity such as particularly silicon carbide bricks, or may be made of the same material in a different manner for example by means of
- 15 ramming and other similar shaping methods either integrally formed in a single piece or in a few large pieces. The insulation of the outer walls of the unheated top portion of the muffle shaft, the so-called charging shaft, greatly promotes the drying and preheating of the charge.

According to the principles of the invention, the middle shaft, formed at the top by the two partitions, is now charged with coarse granular pieces of a material which changes little or nothing in fire, and which may preferably be preheated externally of the charging shaft, for example by the waste heat of the gases from the combustion chamber. The grain size of these pieces is about 20 to about 100 mm. but may be varied within wider limits. These pieces depending on the nature of the zinciferous ore employed may consist of coke, preferably completely degasified, shaped pieces of silicon carbide, porcelain, quartzite stones (coarse gravel), or mixtures of these substances or similar materials. The shape and grain size of this material has to be of such nature that the charge arranged in the middle charging column is as loose and permeable as possible. For example, ring-like spherical, tetrahedron and cube-shaped bodies, or bodies or lumps having angular edges may be employed having approximately equal piece size.

The two laterally disposed charging shafts of the subdivided upper portion of the muffle are charged with a mixture of ore and carbonaceous reducing agent such as is customary for horizontal muffles, although any other desired zinciferous material such as roasted ore, zinc ash, zinc oxide or a mixture of these substances with the usual reducing agent, for example small coke of a suitable grain size, may be employed as a charge material with equal or similar results. The charging openings or ports may be closed in the conventional manner. The muffle is emptied at its bottom end, for example by means of a cooled iron attachment having dimensions corresponding to the cross section of the muffle or in any other conventional manner. At this point both the ash to be removed from the lateral charging columns and the stable or inert material from the middle charging column are withdrawn at a uniform rate. The coarse-grained material from the middle charging column can be constantly recovered by sifting and may be returned to the column and used over again. The removal of the burnt out charge from the iron attachment is carried out continuously or intermittently by mechanical means, for example rollers, or manually. The thickness of the charging columns of coal and ore sliding down the longitudinal walls of the muffle must be so selected that complete burning out is ensured for the selected muffle height and furnace temperature. Generally speaking, thicknesses of

75 about 10 to about 20 cm. have been satisfactory

in practical operation. The middle column of loosely packed stable coarse-grained material has to be so thick that the passage of the zinc vapors is rendered possible at any point of the muffle from the side columns into the middle column 5 and within the latter to the outlet pipe into the condenser, for example upwards. As a rule, a thickness of about 20 to about 40 cm. will be sufficient.

The thermal efficiency of the process of the present invention is a great deal better than in any of the conventional processes. In consequence of the more intimate contact, the ore-coal mixture conducts the heat better and it is also unnecessary to heat the middle of the muffle 15 shaft to the same temperature as the outer wall of the muffle, because the material of the middle core is not metalliferous but has a temperature which permits the zinc vapor to escape unhindered upwards into the condenser. Therefore, 20 it is unnecessary to build the heated muffle shaft very high. As a rule, a heated muffle height of about 4 meters is sufficient. The length of the muffle may be the usual, for example, about 1.5 to about 3 meters. In the structure of the character described it is also possible to effect the removal of deposits, bridge formations and the like in the muffle shaft by means of iron tools 25 or rods from the charging platform without the necessity of temporarily interrupting the operation of the muffle. Due to the fact that the process of the invention does not require briquetting or any other special preliminary treatment of the charge, the cost of smelting and the initial cost of the plant are greatly reduced and the 30 process of the invention can be utilized with equal success for treating any raw materials encountered in practical operation.

In order that those skilled in the art may have a better understanding of the invention, 40 the invention will now be more fully described reference being had to the accompanying drawing which illustrates diagrammatically and by way of example a preferred embodiment of an apparatus suitable for carrying the process of 45 the invention into practice.

Referring now more particularly to Figs. 1 and 2 of the drawing, a bottom structure *a* is carried by a plurality of beams and supports furnace *b* having a heating chamber *b*-1 and a cover *c*. In heating chamber *b*-1 is located a reduction chamber *d* of quadrangular cross-section constituted of silicon carbide in the form of bricks or other shapes. The reduction chamber extends upwards through cover *c* and has its lower end resting on a base *d*-1 supported by the bottom structure *a*. The lower end of the reduction chamber is connected to a discharge shaft *m*, constituted of iron. The upper portion of reduction chamber *d* and extending beyond cover *c* is protected by insulating walls *f* from excessive radiation of heat. This upper portion of the reduction chamber is divided into three compartments by means of two internal partition walls *g*. Of these three compartments, the lateral chambers *h*-1 and *h*-2 are located towards the outside, and a third chamber *i* is formed between the partition walls and in the middle. Partition walls *g* rest on flat arches *e* the supports of which are carried by an anchoring *l* mounted on cover *c* of the furnace. An opening or port *k* is provided in middle chamber *i*, and is connected to a condenser *n* for the zinc vapors. Chamber *i* is closed at the top by means of a cover in a gas tight manner. Instead of the cover, other suit- 70

able closure means may be employed or charging devices capable of being closed. Likewise, closure means of similar character may be provided at the top of chambers *h*-1 and *h*-2. However, generally the columns of charge material located in the upper part of said chambers or shafts are themselves sufficient to provide the necessary closure.

From the above description the operation of the improved vertical muffle will be readily understood by those skilled in the art. After the furnace has been heated up, a normal zinciferous reduction charge is introduced into lateral chambers or shafts *h*-1 and *h*-2. The middle shaft *i* is charged with coarse-grained, inert material such as, for example, coarse pieces of coke. Charging of the lateral chambers *h*-1 and *h*-2 and of the middle chamber *i* is continued until the charge will reach up to the upper edge thereof. Reduction chamber *d* is now heated to the usual reducing temperature of zinc-reducing furnaces by means of suitable heating means such as, for example, gas burners provided in the heating chamber *b*-1. As the zinciferous reduction mixture is in direct contact with the heated walls of reduction chamber *d*, they will be heated by these to a high temperature, whereas the middle portion of chamber *d* down to its bottom is constituted of coarse grained coke sinking downwards from chamber *i*. The furnace heat will cause reduction of the zinciferous material. The zinc vapors liberated thereby and the carbon monoxide gas produced during the reduction will enter the middle zone of coke pieces which is permeable to gases, and will rise unhindered until they arrive through port *k* into condenser *n*. In the condenser the zinc vapor is condensed to liquid zinc while the carbon monoxide leaves the condensation space and is either combusted when it gets into contact with the outer air or may be recovered for further utilization and treatment. During the reduction, the charge goes down and accordingly new charge material is introduced into chambers *h*-1 and *h*-2 at the top thereof and also new pieces of coke in chamber *i* are added. The residues are intermittently removed through discharge shaft *m*, and their finer parts are separated from the coarse pieces of coke. The pieces of coke are reintroduced into the top of chamber *i*, in view of the fact that they leave the reduction chamber substantially unchanged. In this manner the operation of the vertical muffle is carried out continuously. From time to time, the liquid zinc accumulating in condenser *n* is discharged and is cast into ingots.

Although the present invention has been described in connection with a preferred embodiment thereof in which a quadrangular shaft is subdivided by means of a plurality of vertical partition walls, variations and modifications may be resorted to by those skilled in the art without departing from the principles of the present invention. Thus, instead of dividing the top portion of a reducing chamber of rectangular cross section into three shafts, it is also possible to provide a reducing chamber of circular, oval or polygonal cross section in which a corresponding central chamber is divided off by a cylindrical, oval or polygonal member filled with a suitable inert material in coarse lump form. In this case, this middle shaft is enclosed by an annular chamber, or a chamber corresponding in cross section to that of the muffle, to hold the reduction mixture. All of these variations and modifica-

tions are considered as within the true spirit and scope of the present invention as disclosed in the present description and defined by the appended claims.

I claim:—

1. The process for the continuous production of zinc in vertical reducing chambers which comprises establishing a central vertical column constituted of coarse refractory non-sludging lumps of a material not substantially attacked during reduction, establishing vertical columns of a mixture of zinciferous material and reducing agent in proximity to said central column, separating only the upper portions of said vertical columns from each other to prevent direct contact of said upper portions and to establish direct contact of their lower portions, heating said columns to zinc reducing temperatures, passing the zinc vapors produced through said permeable central column, and condensing said zinc vapors. 5 10 15 20

2. The process for the continuous production of zinc in vertical reducing chambers which comprises establishing a central vertical column constituted of coarse refractory non-sludging lumps of a material not substantially attacked during reduction, establishing vertical columns of a mixture of zinciferous material and reducing agent in proximity to said central column separating only the upper portions of said vertical columns from each other to prevent direct contact of said upper portions and to establish direct contact and communication between their lower portions, heating said columns to zinc-reducing temperatures, passing the zinc vapors produced through said permeable central column, and condensing said zinc 25 30 35 vapors.

3. The process for the continuous production of zinc in vertical reducing chambers which comprises establishing a central vertical column constituted of coarse refractory non-sludging lumps 40 of a material not attacked by zinc vapors, establishing lateral vertical columns of a mixture of zinciferous material and reducing agent in proximity to said central column, separating only the upper portions of said vertical columns from each 45 other to prevent direct contact of said upper portions and to establish direct contact, intimate heat exchange and communication between their lower portions, applying heat to the lower portion of said central column to heat said columns 50 to zinc-reducing temperatures, continuously withdrawing zinc vapors produced through said central column permeable to gases, and condensing said zinc vapors.

4. The process for the continuous production 55 of zinc in vertical reducing chambers which comprises establishing a central vertical column constituted of coarse refractory non-sludging lumps of a material not attacked by zinc vapors, establishing at least one lateral vertical column of a 60 mixture of zinciferous material and reducing agent in proximity to said central column, separating only the upper portions of said vertical columns from each other to prevent direct contact of said upper portions and to establish direct 65 contact, intimate heat exchange and communication between their lower portions, heating said columns to zinc-reducing temperatures, continuously withdrawing zinc vapors through said permeable central column, condensing said zinc vapors, introducing fresh charge materials into said columns at the top thereof, and removing solid residual products at the bottom of said central shaft. 70

5. The process for the continuous production 75

of zinc in vertical reducing chambers which comprises establishing a central vertical column of coarse refractory non-slagging lumps of a material not substantially attacked during reduction, 5 establishing vertical columns of a mixture of zinciferous material and reducing agent in proximity to said central column, separating only the upper portions of said vertical columns from each other to prevent direct contact of said upper portions and to establish direct contact, intimate heat exchange and communication between their lower portions, applying indirect heat to the lower portion of said vertical reducing chamber to cause reduction of the zinciferous materials to metallic 10 zinc, withdrawing zinc vapors and reduction gases through said permeable central column, condensing said zinc vapors, feeding fresh charge materials into said columns at the top thereof, and removing residual products at the bottom of said 15 central column.

6. The process for the continuous production of zinc in vertical reducing chambers which comprises establishing a central vertical column of coarse refractory non-slagging lumps of a material not attacked by zinc vapors and having a grain size of about 20 to about 100 mm., establishing vertical columns of a mixture of zinciferous material and reducing agent in proximity to said central column, separating only the upper 20 portions of said vertical columns from each other to prevent direct contact of said upper portions and to establish direct contact, intimate heat exchange and communication between their lower portions, applying indirect heat to the lower portion of said vertical reducing chamber to cause reduction of the zinciferous materials to metallic zinc, withdrawing zinc vapors and reduction gases through said permeable central column, condensing said zinc vapors, feeding fresh charge 25 materials into said columns at the top thereof, removing residual products at the bottom of said central column, recovering the coarse lumps of the central column from said residual products by sifting, and returning the same to said vertical column for further use.

7. A vertical muffle for the continuous production of zinc comprising a vertical reducing shaft, a heating chamber externally surrounding the lower portion of said shaft, partition walls dividing the upper portion of said shaft into vertical central and lateral chambers, a port at the top of said central chamber to introduce coarse refractory non-slagging lumps of a material not substantially attacked during reduction, openings at the top of said lateral chambers to fill the same with a mixture of zinciferous material and reducing agents, heating means in said heating chamber to heat said vertical reducing shaft to zinc-reducing temperatures, and a port at an intermediate portion of said central chamber to withdraw zinc vapors therefrom.

8. A vertical muffle for the continuous production of zinc comprising a vertical reducing shaft constituted of a highly refractory structural material having good heat conductivity, a heating chamber externally surrounding the lower portion of said shaft, partition walls within said shaft dividing the upper portion thereof into a vertical central chamber and a pair of lateral chambers, a port at the top of said central chamber to introduce coarse refractory non-slagging lumps of a material not attacked by zinc vapors, ports at the top of said lateral chambers to fill the same with a mixture of zinciferous material and reducing agents, heating means in said heating

chamber to heat the vertical reducing shaft to zinc-reducing temperatures, and a port in an intermediate portion of said central chamber to withdraw zinc vapors therefrom.

9. A vertical muffle for the continuous production of zinc comprising a quadrangular vertical reducing shaft constituted of a highly refractory structural material having good heat conductivity, a heating chamber externally surrounding the lower portion of said shaft, a pair of partition walls within said shaft dividing the upper portion thereof into a vertical central chamber and a pair of lateral chambers, a pair of arches within said shaft for supporting said partition walls, a port at the top of said central chamber to introduce coarse refractory non-slagging lumps of a material not substantially attacked during reduction thereinto, openings at the top of said lateral chambers to fill the same with a mixture of zinciferous material and reducing agents, heating means in said heating chamber to heat the vertical reducing shaft to zinc reducing temperatures, and a port in an intermediate portion of said central chamber to withdraw zinc vapors therefrom.

10. A vertical muffle for the continuous production of zinc comprising a quadrangular vertical reducing shaft constituted of a highly refractory structural material having good heat conductivity, a heating chamber externally surrounding the lower portion of said shaft, a pair of partition walls within said shaft dividing the upper portion thereof into a vertical central chamber and a pair of lateral chambers, a pair of arches within said shaft for supporting said partition walls, a port at the top of said central chamber to introduce coarse refractory non-slagging lumps of a material not attacked by zinc vapors thereinto, ports at the top of said lateral chambers to fill the same with a mixture of zinciferous material and reducing agents, heating means in said heating chamber to heat the vertical reducing shaft to zinc reducing temperatures, a port at an intermediate portion of said central chamber to withdraw zinc vapors therefrom, and a condenser connected to said port to condense said vapors.

11. A vertical muffle for the continuous production of zinc comprising a vertical reducing shaft constituted of a highly refractory structural material having good heat conductivity, a heating chamber externally surrounding the lower portion of said shaft, a cover for said heating chamber having said shaft protruding therethrough, a pair of partition walls within said shaft dividing the upper portion thereof into a vertical central chamber and a pair of lateral chambers, a pair of arches within said shaft for supporting said partition walls, a charging port at the top of said central chamber to introduce coarse refractory non-slagging lumps of a material not attacked by zinc vapors thereinto, charging ports at the top of said lateral chambers to fill the same with a mixture of zinciferous material and reducing agents, closure means for said charging ports, heating means in said heating chamber to heat said vertical chambers to zinc-reducing temperatures, a discharge port in an intermediate portion of said central chamber to withdraw zinc vapors therefrom, a condenser for condensing said vapors, and a discharge shaft connected to the bottom end of said vertical shaft for the removal of residual materials.